

April 22, 1930.

E. O. BARSTOW

1,755,380

METHOD AND MEANS FOR ELECTROLYTIC PRODUCTION OF LIGHT METALS

Filed Nov. 9, 1925



Fig. 1.



Fig. 2

INVENTOR.  
Edwin O. Barstow  
BY  
Day, Oberlin & Day  
ATTORNEYS.

## UNITED STATES PATENT OFFICE

EDWIN O. BARSTOW, OF MIDLAND, MICHIGAN, ASSIGNOR TO THE DOW CHEMICAL COMPANY, OF MIDLAND, MICHIGAN, A CORPORATION OF MICHIGAN

## METHOD AND MEANS FOR ELECTROLYTIC PRODUCTION OF LIGHT METALS

Application filed November 9, 1925. Serial No. 67,780.

In the electrolytic production of metallic magnesium, by passing an electric current through a suitable fused electrolyte, one of the difficulties encountered is the collection of the separate molten globules of the metal. These, as they are set free, rise to the surface due to their lighter specific gravity, but do not readily coalesce, at least until a considerable mass of the molten metal has accumulated.

The object of the present invention is to provide an improved method and apparatus whereby such free molten globules of the metal may be positively collected together at a selected point in the electrolytic cell, thus facilitating the removal or discharge of the metal.

To the accomplishment of the foregoing and related ends, the invention then consists of the steps and means hereinafter described and particularly pointed out in the claims, the annexed drawing and following description illustrating but several of the various ways in which the principle of the invention may be carried out.

In said annexed drawing:—

Fig. 1 is a more or less diagrammatic plan view of one type of electrolytic cell such as is used in the production of metallic magnesium, the construction of such cell being modified to adapt the same for the collecting together of the molten metal in accordance with the present invention; and Fig. 2 is a vertical section of such cell, partly on an axial plane and partly on a plane in front of such axial plane, as indicated by the line 2—2, Fig. 1.

The principal element in the apparatus illustrated in the drawing is a cast iron or steel vessel (1) that constitutes the cell proper and in which the electrolyte is placed and maintained in molten condition. This vessel at the same time constitutes the cathode and, for the purpose of initially melting the electrolyte, the vessel may be supported in a suitable furnace chamber (not shown).

Supported in any suitable way within vessel 1 is an annular diaphragm or partition (2) of porcelain, fire clay, or equivalent material that serves to laterally surround the centrally

disposed, depending carbon or graphite anode (3). Neither the latter, nor such annular diaphragm extends entirely down to the bottom of the vessel. The anode, however, extends downwardly beyond the lower edge of the diaphragm. A suitable duct, not shown, may be provided if desired for supplying the electrolyte to the cathode compartment of the cell, i. e., that portion lying between the wall of the vessel (1) and the annular diaphragm (2); while a duct (4) is connected with the upper portion of the space within the diaphragm in order to conduct away any gases arising from the anode compartment defined by such diaphragm.

In the operation of a cell such as the foregoing, the particles of free molten magnesium, many quite small in size, rise to the surface of the electrolyte in the aforesaid cathode compartment, and there float as separate globules which do not readily coalesce and, at the best, form a thin film only of the metal, which is difficult to remove either by dipping or through a spout or equivalent discharge opening. The present improvement consists as previously indicated in the provision of means for collecting these free molten globules of metal and in the preferred form illustrated, such means comprise a box-like chamber (5), lying between the diaphragm (2) and the wall of vessel (1). The respective end walls of this chamber are submerged below the bath level, but the lateral walls rise well above such level. Two transverse partitions (6) and (7) in said chamber (5) form a sub-compartment (8) that is open both above and below. The second of these partitions (see Fig. 2), it will be noted, extends downwardly further than the first and in the portion (9) of the chamber adjacent to the sub-compartment (8) there is located a propeller (10) carried by an externally driven vertical shaft (11), such propeller serving when operated to induce a flow of the electrolyte through the several compartments of chamber (5) in the direction indicated by the arrows.

Only the upper stratum of the electrolyte lying between the annular partition (2) and the surrounding wall of vessel (1) will be af-

55

60

65

70

75

80

85

90

95

100

fected, and, depending upon the size and rate of rotation of propeller (10) this stratum may be circulated at any desired rate of speed so as to be entirely caused to pass through chamber (5) within a stated time. Due to the arrangement of the transverse partitions (6 and 7) within the chamber, as clearly shown in Fig. 2, the particles or globules of molten metal are entrapped in the sub-compartment defined by said partitions and are there collected together to form a mass of molten metal of substantial thickness. From this sub-compartment the metal may be removed either by dipping or a suitably controlled laterally opening sprue or discharge spout may be provided to conduct the metal from said compartment to a point without the cell.

It will be understood that the propeller (10) may be operated either continuously or intermittently. Thus, it may be found satisfactory to induce a circulation of the upper stratum of the electrolyte in the manner hereinbefore described at intervals only. In that event, the propeller will simply remain idle except when it is desired to collect together the molten metal that has been produced by the electrolysis of the bath. Various equivalent mechanical and other means may of course be employed to induce the circulation of the electrolyte in the manner hereinbefore described and, similarly, I do not limit myself to any precise form of trap chamber for collecting together the globules or particles of molten metal as they are thus carried around by the circulating electrolyte.

Other modes of applying the principle of my invention may be employed instead of the one explained, change being made as regards the means and the steps herein disclosed, provided those stated by any of the following claims or their equivalent be employed.

I therefore particularly point out and distinctly claim as my invention:—

45 1. The method of aggregating light metal floating on a fused electrolyte, which comprises mechanically circulating said electrolyte through a trapped zone in which the floating metal is arrested.

50 2. In a method of electrolyzing a fused electrolyte for the production of a metal which will float thereon, the step which comprises mechanically circulating the surface portion of said electrolyte through a trap adapted to arrest metal floating thereon.

55 3. A method of electrolyzing a fused electrolyte containing magnesium chloride for the production of magnesium metal, which comprises mechanically circulating the surface layer of said electrolyte through a trap adapted to arrest and retain such floating metal.

4. A method of producing a light metal which comprises electrolyzing a suitable fused electrolyte, mechanically driving the

upper stratum of such electrolyte about in an approximately circular surface path, and entrapping at one point the free molten globules of metal therein.

5. In a method of electrolyzing a fused electrolyte for the production of a metal which will float thereon, the step which comprises liberating said metal as such, permitting it to rise to the surface of the electrolyte, and collecting such metal by mechanically circulating the electrolyte upon which it floats through a trapped zone.

6. In an electrolytic apparatus for liberating a light metal upon a non-fluid cathode from a fused electrolyte heavier than the metal liberated, the combination with a vessel adapted to contain the fused electrolyte, of means to mechanically circulate said electrolyte through a trap within said vessel to arrest metal floating on said electrolyte.

7. In an electrolytic apparatus for liberating a light metal upon a non-fluid cathode from a fused electrolyte heavier than the metal liberated, the combination with a vessel adapted to contain the fused electrolyte and act as cathode, of an anode depending in said electrolyte, means to separate products liberated upon the anode from those liberated upon the cathode, and mechanical means to circulate the catholyte through a trap to skim and arrest metal floating upon the surface.

8. In an electrolytic apparatus for producing a metal lighter than the electrolyte, the combination of a vessel adapted to contain a fused electrolyte, means for passing an electric current therethrough, means for positively driving in a surface circuit the portion of such electrolyte containing free molten globules of metal, and a trap located in such circuit to collect the globules together.

9. In an electrolytic apparatus for producing a metal lighter than the electrolyte, the combination of a vessel of general circular form adapted to contain a fused electrolyte and constituting one electrode, a second electrode disposed approximately centrally within said vessel, means for driving the upper stratum of such electrolyte around said second electrode, and a trap-chamber within said vessel disposed in the path of such circulating electrolyte and adapted to collect together the free, molten globules of metal therein.

10. In an electrolytic apparatus for producing a metal lighter than the electrolyte, the combination of a vessel of general circular form adapted to contain a fused electrolyte and constituting one electrode, a second electrode disposed approximately centrally within said vessel, means adapted to cause a circulation of the upper stratum of such electrolyte around said second electrode, a chamber lying between the wall of said vessel and said second electrode so as to permit

such circulating electrolyte to flow therethrough and having a transverse partition arranged to trap and so collect together the free, molten globules of metal in the electrolyte.

- 5 11. In an electrolytic apparatus for producing a metal lighter than the electrolyte, the combination of a vessel of general circular form adapted to contain a fused electrolyte and constituting one electrode, a second electrode disposed approximately centrally within said vessel, a chamber lying between the wall of said vessel and said second electrode, the end walls of said chamber being 10 submerged so as to permit the upper stratum of such electrolyte to flow thereover, transverse partitions in said chamber forming a sub-compartment open at the top and bottom, and a propeller in said chamber adjacent said 15 sub-compartment.

- 20 12. In an electrolytic apparatus for producing a fused metal lighter than the fused electrolyte employed, the combination with a suitable vessel adapted to contain said fused electrolyte, of a trap disposed within said vessel in said electrolyte to arrest and retain floating metal, and a mechanically driven means in said vessel to circulate the electrolyte upon which the metal floats through said 25 trap.

Signed by me this 6th day of November,  
1925.

EDWIN O. BARSTOW.

35

40

45

50

55

60

65